

1

2,859,181

## HEAT STABLE LITHIUM-LEAD SOAP COMPOSITION

Terence B. Jordan, Fishkill, N. Y., and Oney P. Puryear, Houston, Tex., assignors to The Texas Company, New York, N. Y., a corporation of Delaware

No Drawing. Application May 2, 1956  
Serial No. 582,069

6 Claims. (Cl. 252—62.5)

This invention relates to a heat stable fluid composition which has the ability to retain metals suspended therein. More particularly, this invention relates to a heat stable fluid designed for use as a carrier vehicle for iron in a magnetic clutch.

The heat stable fluid composition of this invention comprises a highly refined mineral lubricating oil having a V. I. of at least 80 as the major component, 2 to 4 weight percent lithium salt of a  $C_{12}$  to  $C_{24}$  hydroxy fatty acid and 0.5 to 2 weight percent of a lead salt of a  $C_{12}$  to  $C_{24}$  hydroxy fatty acid, the total salt concentration falling between 2 and 6 weight percent of the composition. The addition of iron particles to the heat stable composition of this invention produces an excellent magnetic clutch fluid.

The requirements of a fluid to be employed as the power transmitting means in a magnetic fluid clutch are the following: a high viscosity index, a high flash and fire point, low vapor pressure and high temperature stability. The National Bureau of Standards in their development of the magnetic fluid clutch discovered that a highly refined mineral lubricating oil filled these requirements and that a mixture comprising 1 part of a 10 grade paraffin base mineral oil and 5 to 9 parts of finely divided iron, prepared by decomposing iron carbonyl, was a good power transmission fluid. It was soon discovered that iron particles tended to settle out of 10 grade mineral oil during idle periods and caked on the bottom of the housing wherein the magnetic fluid clutch was encased. As a consequence, considerable difficulty in starting was encountered using a mixture of iron particles and 10 grade mineral oil as the power transmitting fluid.

Any material added to the mineral oil to correct its deficiencies in retaining the iron particles in suspended form should have the following properties: (1) It should possess a relatively high gelling temperature. (2) It should be stable on cooling statically from temperatures above the melting point of the added material. (3) It should not increase the transmission of torque due to increased consistency or viscosity of the medium when the clutch is de-energized. In addition, the added material should not adversely affect the previously mentioned properties of high viscosity index, low vapor pressure, high temperature stability and high flash and fire points. The composition of this invention, comprising a mixture of lithium and lead hydroxy fatty acid soaps in a mineral oil, fills all of the above requirements as will be demonstrated hereafter.

Hydroxy fatty acids containing 12 to 24 carbon atoms can be used in the formulation of the lithium and lead salts employed in the composition of this invention. 12-hydroxy stearic acid is usually employed as the lead and lithium soap precursor because of its availability and cost. Hereafter in the description of the invention, 12-hydroxy stearic acid will be used in the production of the lead and lithium soaps. Examples of other hydroxy acids that can be employed are the following: 9-

2

hydroxy stearic acid, 10-hydroxy stearic acid, 9,10-dihydroxy stearic acid, 8-hydroxy myristic acid and 10-hydroxy palmitic acid.

In order for the composition of this invention to be effective as a medium for maintaining iron particles in suspension, the concentration of the lithium plus lead hydroxy stearates must fall between 2 and 6 weight percent. At soap concentrations below 2 weight percent, the mixture does not maintain the iron particles in suspended form. If the total concentration of lithium and lead hydroxy stearates is greater than 6 weight percent, the consistency of the fluid vehicle is too high with the result that the transmission of torque, particularly during start up, is adversely affected. The preferred concentration of the lithium plus lead soaps falls between 3 and 5 weight percent.

The lithium hydroxy stearate usually is present in an amount between 2 to 4 weight percent of the vehicle composition while the lead hydroxy stearate constitutes 0.5 to 2 weight percent of the vehicle. The ratio of lithium hydroxy stearate to lead hydroxy stearate falls between 2 and 4. The preferred composition comprises the lithium and lead hydroxy stearates in a weight ratio of 3:1. A composition containing 3 weight percent lithium hydroxy stearate and 1 weight percent lead hydroxy stearate has proven extremely effective in an extended run in an experimental magnetic fluid clutch.

The mineral lubricating oil component of the composition of this invention must have a V. I. of at least 80 and an SUS viscosity at 100° F. above 150. An SAE 10 grade paraffin base distillate oil, which has been solvent refined to remove low V. I. materials and solvent dewaxed to remove waxy particles to improve its pour, fills these requirements and is the preferred base oil for the composition of this invention. In general, any distillate lubricating oil fraction having a V. I. above 80, an SUS viscosity at 100° F. above 150 and a flash above 350° F. can be employed as the mineral lubricating oil component of the fluid composition of this invention.

The composition of this invention can be prepared by the addition of the prescribed amounts of lithium and lead hydroxy stearates thereto, but it has been found more convenient to form the lithium and lead soaps in situ by a process involving saponification of the hydroxy stearic acid by lead oxide and lithium hydroxide in the mineral lubricating oil base and subsequent dehydration of the saponified mixture.

A preferred procedure for forming the fluid composition of this invention is described in the copending application, Serial No. 582,068, filed of even date. In the copending application there is disclosed a process for obtaining improved yields of compositions, particularly greases, containing a mixture of lithium and lead hydroxy fatty acid soaps. The procedure for obtaining improved yields of a soap-thickened composition containing a mixture of lithium and lead hydroxy fatty acid soaps comprises adding the hydroxy fatty acid to a portion of the mineral oil base, separate formation of the lead hydroxy fatty acid soap by saponification at a temperature above 280° F. and dehydration at a similar temperature, subsequent formation of the lithium hydroxy fatty acid soap by saponification at a temperature of approximately 200° F. followed by dehydration at a temperature above 280° F. This procedure was employed in the formation of the compositions of this invention.

The effectiveness of various compositions for suspending iron was determined in the laboratory by a procedure involving the addition of about 85% by weight of iron powder to the vehicle and evaluation of the mixture after a uniform mixture had been formed by stirring at room temperature. 50 ml. of uniform iron-vehicle mixture under test was heated to an elevated temperature with stirring, transferred to a 50 ml. graduate and al-

lowed to stand undisturbed for an extended period. The volume of separated oil was recorded at regular intervals and the amount of separation against time was determined for each system. Powdered iron-mineral oil vehicles were used as a standard. The determinations were made after one cycle of heating, after 12 cycles of heating, or after both 1 and 12 cycles. The 12 cycle measurement more closely simulates the magnetic clutch operation.

A number of compositions containing different concentrations of lithium and lead 12-hydroxy stearates were prepared according to the procedure defined in the afore-identified copending application. The effectiveness of these compositions in retaining finely divided iron particles in suspension is shown in the following table in comparison with compositions containing other common suspending agents such as aluminum stearate, polyethylene glycol oleate and calcium naphthenate.

TABLE I.

*Suspending power of stabilized mineral oil compositions for iron powder*

|                                                                                           | ML. of Oil Separated from 50 ml. of Composition Containing 85% Iron Powder |                |
|-------------------------------------------------------------------------------------------|----------------------------------------------------------------------------|----------------|
|                                                                                           | 1 Cycle                                                                    | 12 Cycles      |
| <b>Iron Powder In:</b>                                                                    |                                                                            |                |
| Base Oil A.                                                                               | 18 in 220 Hrs.                                                             | 17 in 250 Hrs. |
| Base Oil A containing 1.5% lithium 12-hydroxy stearate and 0.5% lead 12-hydroxy stearate. | 10 in 216 Hrs.                                                             | 8 in 64 Hrs.   |
| Base Oil A containing 3% lithium 12-hydroxy stearate and 1% lead 12-hydroxy stearate.     | 0 in 220 Hrs.                                                              | 0 in 250 Hrs.  |
| Base Oil A containing 12% calcium naphthenate.                                            | 1 in 56 Hrs.                                                               | 2 in 250 Hrs.  |
| Base Oil B.                                                                               | 16 in 72 Hrs.                                                              |                |
| Base Oil B containing 3% lithium 12-hydroxy stearate and 1% lead 12-hydroxy stearate.     | 0 in 72 Hrs.                                                               |                |
| Base Oil B containing 2% polyethylene glycol monooleate.                                  | 10 in 72 Hrs.                                                              |                |
| Base Oil B containing 12% calcium naphthenate.                                            | 1.5 in 72 Hrs.                                                             |                |
| Base Oil B containing 3% aluminum stearate.                                               | 11 in 72 Hrs.                                                              |                |

Base Oil A employed in the compositions of the previous table is a furfural refined, solvent dewaxed, paraffin base distillate oil having SUS viscosities at 100 and 210° F. of 185 and 50, respectively, a viscosity index of 110, a pour of -20° F. and a flash above 420° F. Base Oil B is a furfural refined, solvent dewaxed, paraffin base distillate oil having SUS viscosities at 100 and 210° F. of 165 and 50, respectively, a viscosity index of 100, a pour of -15° F. and a flash above 400° F.

The data in the foregoing table demonstrate that a composition comprising a refined distillate oil and 2 to 5 weight percent of a mixture of lithium and lead 12-hydroxy stearates is an excellent vehicle for maintaining finely divided iron particles in suspension. The data show clearly that substantial improvement of the base oil is obtained with a concentration of 2 weight percent of lithium and lead 12-hydroxy stearates, but that much superior results are obtained when the total soap concentration falls within the preferred concentration range of 3 to 4.5 weight percent.

The calcium naphthenate-containing composition also showed good effectiveness in retaining iron particles in suspension. Although aluminum stearate and polyethylene glycol oleate (glycol having average molecular weight of 400) improved the ability of the base oil to retain iron particles in suspension, neither was considered an effective additive.

Since both calcium naphthenate and the mixture of lithium and lead 12-hydroxy stearates were effective in retaining iron powder in suspension, compositions containing these additives were scheduled for evaluation in

a magnetic fluid clutch. Before the composition comprising Base Oil A, 12% calcium naphthenate and iron powder could be evaluated, the iron particles separated from the oil with the result that it was not evaluated.

5 However, the composition comprising Base Oil A, 3% lithium 12-hydroxy stearate, 1% lead 12-hydroxy stearate and iron powder was run in a magnetic fluid clutch for 400 hours with outstanding results. The amount of iron powder in each evaluation was approximately 7 parts by weight. Although the magnetic clutch was subjected to frequent stops and starts, no difficulty was encountered in start-up. There was no evidence of settling of iron particles in the bottom of the housing encasing the magnetic fluid clutch.

10 15 The composition of this invention comprising a highly refined distillate oil having a V. I. above 80 and an SUS viscosity at 100° F. above 150, 2 to 5 weight percent lithium hydroxy stearate and 0.5 to 2 weight percent lead hydroxy stearate, the total salt concentration falling between 2 and 5 weight percent, is an outstanding vehicle for iron powder. When magnetic fluid clutches attain greater commercial use, this fluid vehicle in combination with 5 to 9 parts by weight of finely divided iron, is expected to be widely used.

20 25 Obviously, many modifications and variations of the invention, as hereinbefore set forth, may be made without departing from the spirit and scope thereof and, therefore, only such limitations should be imposed as are indicated in the appended claims.

30 We claim:

1. A heat stable composition consisting essentially of a liquid vehicle comprising a highly refined mineral lubricating oil having a V. I. of at least 80 as the major component, 2 to 4 weight percent lithium salt of hydroxy stearic acid, and 0.5 to 2 weight percent of the lead salt of hydroxy stearic acid, the total concentration of said lithium and lead salts being not more than 6 weight percent and not less than 2 weight percent and finely divided iron powder in an amount between 5 and 9 parts by weight of said liquid vehicle.

35 40 2. A heat stable composition according to claim 1 containing 3 weight percent lithium 12-hydroxy stearate and 1 weight percent lead 12-hydroxy stearate.

3. A heat stable composition according to claim 1 in which the weight ratio of said lithium 12-hydroxy stearate to lead 12-hydroxy stearate falls between 2 and 4.

45 4. A heat stable composition according to claim 1 in which said lubricating oil has an SUS viscosity at 100° F. above 150, and a flash above 350° F.

50 55 5. A composition for use as a magnetic clutch fluid consisting essentially of a liquid vehicle comprising a highly refined mineral lubricating oil having a V. I. of at least 80, 2 to 4 weight percent lithium 12-hydroxy stearate, 0.5 to 2 weight percent lead 12-hydroxy stearate, the total concentration of said lithium and lead 12-hydroxy stearates being not more than 6 weight percent and not less than 2 weight percent, and finely divided iron powder in an amount between 5 and 9 parts by weight of the liquid vehicle.

60 65 6. A composition for use as a magnetic clutch fluid consisting essentially of a liquid vehicle comprising an SAE 10 grade paraffin base mineral oil having a viscosity index above 80, 3 weight percent lithium 12-hydroxy stearate, 1 weight percent lead 12-hydroxy stearate and finely divided iron powder in an amount between 5 and 9 parts by weight of said liquid vehicle.

#### References Cited in the file of this patent

#### UNITED STATES PATENTS

- |           |              |                |
|-----------|--------------|----------------|
| 2,106,882 | Betz         | Feb. 1, 1938   |
| 2,308,599 | Fraser       | Jan. 19, 1943  |
| 2,652,366 | Jones et al. | Sept. 15, 1953 |
| 2,661,596 | Winslow      | Dec. 8, 1953   |